

# United States Patent [19]

Erickson

[11] 3,846,881

[45] Nov. 12, 1974

[54] FILAMENT CRIMPING

[75] Inventor: Wayne K. Erickson, Greenville, S.C.

[73] Assignee: Phillips Petroleum Company,  
Bartlesville, Okla.

[22] Filed: Jan. 5, 1972

[21] Appl. No.: 215,461

[52] U.S. Cl. 28/72.14

[51] Int. Cl. D02g 1/12

[58] Field of Search 28/1.6, 1.2, 1.3, 72.1,  
28/72.11, 72.14, 72.17, 1.5; 19/65 T, 66 T;  
264/168, 282; 57/140 B, 157 S

## [56] References Cited

### UNITED STATES PATENTS

2,810,281 10/1957 Appleton et al. 28/72.17 X  
3,039,171 6/1962 Hume et al. 28/72.17

|           |         |                        |            |
|-----------|---------|------------------------|------------|
| 3,115,744 | 12/1963 | Nott.....              | 57/157 S   |
| 3,175,348 | 3/1965  | Bloch.....             | 28/1.5     |
| 3,199,281 | 8/1965  | Maerov et al. ....     | 57/140 B   |
| 3,234,624 | 2/1966  | Shattuck.....          | 28/1.6     |
| 3,384,932 | 5/1968  | Watson.....            | 19/65 T    |
| 3,387,349 | 6/1968  | Trifunovic et al. .... | 28/72.14 X |
| 3,408,251 | 10/1968 | Davies et al. ....     | 28/72.17 X |
| 3,423,809 | 1/1969  | Schmitt.....           | 28/72.17   |
| 3,601,872 | 8/1971  | Potman et al. ....     | 28/1.3     |
| 3,653,198 | 4/1972  | Hopkins.....           | 28/72.17   |
| 3,681,821 | 8/1972  | Buck.....              | 28/1.3     |

Primary Examiner—Louis K. Rimrodt

## [57] ABSTRACT

Two separate filament structures are crimped simultaneously but at different temperatures to produce a combined filament structure having two levels of crimp.

4 Claims, 1 Drawing Figure



PATENTED NOV 12 1974

3,846,881



INVENTOR.  
W. K. ERICKSON

BY

*Dugg & Oberlin*

ATTORNEYS

## FILAMENT CRIMPING

## BACKGROUND OF INVENTION

This invention relates to a method and apparatus for crimping filament structures and to the crimped product.

Often it is desirable to crimp synthetic filament structures to increase the bulk and cover, improve the hand, etc. In many instances it is preferred to avoid having the crimp in register, that is having the crimp loops of individual filaments aligned with loops of other filaments. When making staple fibers from continuous filaments it is not unusual to crimp the filaments prior to chopping into staple lengths. It is desirable that such crimped staple have good card web adhesion.

An object of my invention is to produce crimped filament structures. Another object of my invention is to produce crimped staple which has good card web adhesion. Another object of my invention is to produce crimped yarn while avoiding complete register of the crimp.

## SUMMARY OF INVENTION

I have found that crimped filament structures can be made by simultaneously stuffer crimping in one crimpler at least two portions of the structure which are at different temperatures when fed to the crimpler. Further according to my invention a single filament structure is divided into at least two portions and one portion is heated before feeding to the crimpler. Further according to my invention a filament structure produced by simultaneous crimping of at least two portions of the structures at different temperatures in a single crimpler, is chopped to produce crimped staple fibers.

My invention also includes apparatus for performing the process described above and the resulting products.

## DETAILED DESCRIPTION

In the drawing a stuffer crimpler 11 comprises crimpler rolls 12 and 13, inlet guide 14 and body 16. A heater 17 is provided in the path of the portion of the feed to the crimpler, and guide rolls 18 and 19 are provided in a separate path to the crimpler. Guide rolls 20 and 21 are provided for the combined filament structure.

In operation a tow 22 passes over guide roll 20, is divided into two filament structure portions 23 and 24. Portion 23 passes over heater 17 and then to guide roll 21 while portion 24 passes around guide rolls 18 and 19 through a path in which it is not subjected to heating by heater 17. Portions 23 and 24 are recombined on guide roll 21 and fed into stuffer crimpler 11. The crimped product from crimpler 11 is removed therefrom for further handling as desired and necessary. This can include for example takeup rolls for packaging or the yarn can be sent directly to further processing, for example, chopping to produce staple fibers.

## EXAMPLE

In an example according to my invention, utilizing the apparatus described above, a 5,000 denier, 280 filament, drawn polypropylene tow was supplied to stuffer crimpler 11 having one-fourth inch face width crimpler rolls, at 40 meters per minute. One-half of the tow

(2,500 denier) was routed over heater 17 which was a draw shoe type surface heater with temperature control and controlled at 400°F. surface temperature. The other half of the tow (2,500 denier) was passed over guide rolls 18 and 19 out of contact with heater 17. The two halves were recombined at roll 21 and were crimped in crimpler 11. The resulting crimped tow had two distinct crimp levels.

For comparison, holding the stuffer box pressure and the crimpler roll pressure constant, the portion of the tow passing over heater 17 was guided away from the surface thereof whereby the two portions of the tow were fed to crimpler 11 at substantially the same temperature. The resulting tow had near uniform, one level crimp.

This example illustrates the effectiveness of the apparatus and method according to my invention to produce a crimped tow having two levels of crimp and demonstrates further that this result is not obtained merely by dividing the tow into two parts without heating one of the parts.

Throughout the application and in the claims the term "filament structure" has been used to include all crimpable filaments including yarns, tows, slivers, rovings, etc. The material from which the filaments are made can be any material which produces crimpable filaments including, for example, polypropylene, nylon, polyester, etc.

Reasonable variation and modification are possible within the scope of my invention. For example, means other than surface heaters can be used for heating one portion of the filament structure including such means as radiant heaters, contact with heated fluid, etc. Means other than the guide rolls can be used for providing the separate paths for the filament portions. The temperatures of the two portions which are combined and fed to the crimpler can vary widely depending upon the condition of the structure to be processed and the results desired. The cooler of the two portions can be at ambient temperature or can be below or above ambient temperature. The temperature of the warmer portion should be sufficiently above that of the cooler portion to give the desired variation in crimp level and the resulting product. In general, the larger the temperature differential the more noticeable will be the resulting two crimp level in the product. Although the invention has been described and presently finds its greatest application in systems in which the feed to the crimpler is divided into only two parts, the invention also is applicable to systems in which the feed is divided into three or more portions at different temperature levels.

The term "crimp level" in this application is used to mean crimp frequencies and amplitudes as well as the nature of the crimping, i.e., the shape of the crimp loops, and a variation in crimp level can be in any one or more of these elements of crimp. For example, two crimp levels are obtained when two crimp frequencies are obtained even though the amplitude may be substantially the same. However, more commonly, when practicing my invention differences in both frequency and amplitude result.

What is claimed is:

1. A method of producing a crimped filament structure comprising passing a first portion of said filament structure into a stuffer crimpler at a first temperature;

simultaneously passing a second portion of said filament structure into said stuffer crimper at a second temperature substantially higher than said first temperature; and

simultaneously subjecting said first portion and said second portion to crimping conditions in said stuffer crimper thereby producing a filament structure having crimp variations between individual filaments thereof.

2. A method of producing a filament structure comprising dividing a filament structure into a first portion and a second portion;

heating said second portion to a temperature substantially above the temperature of said first portion;

5

10

15

recombining said first and second portions; and passing said recombined portions to a stuffer crimper whereby said first and second portions are simultaneously subjected to crimping conditions at substantially different temperatures producing a filament structure having crimp variations between individual filaments thereof.

3. The method of claim 2 wherein

said filament structure having crimp variations is cut to produce staple fibers.

4. The method of claim 2 wherein said second portion of filament structure is heated by passing said second portion in proximity to heating means.

\* \* \* \* \*

20

25

30

35

40

45

50

55

60

65